

Jan. 14, 1958

C. ALBRECHT

2,819,992

CARBURIZATION OF IRON AND STEEL

Filed April 27, 1956



Fig. 1.



BY

Bailey, Stephens & Heietig  
ATTORNEYS

1

2,819,992

## CARBURIZATION OF IRON AND STEEL

Carl Albrecht, Kronberg, Germany, assignor to Deutsche Gold- und Silber-Scheideanstalt vormals Roessler, Frankfurt am Main, Germany

Application April 27, 1956, Serial No. 581,126

Claims priority, application Germany April 27, 1955

3 Claims. (Cl. 148—15.5)

The present invention relates to improvements in the carburization of ferrous metals, such as iron and steel, in a salt bath essentially consisting of halides and cyanides, especially at temperatures higher than previously customarily employed and to salt baths for carrying out such process.

The cementation of iron or steel articles in fused salt baths containing cyanides to carburize such articles to a certain depth beneath their surface is already known. The fused salt baths used for this purpose contain alkali metal and/or alkaline earth metal halides and one or more cyanides as their essential constituents. The decrease of the carbon content with increase in depth from the surface of the article carburized and the required duration of the carburization treatment primarily depend upon the cyanide content of the bath employed, the presence of accelerators and also the temperature employed for the carburization. With baths which do not contain accelerators which generally contain more than 40% of cyanide, one usually obtains cases having a relatively low carbon content. Furthermore, such baths are normally used at relatively low temperatures of about 700 to 800° C.

In salt baths containing additions which accelerate the delivery of carbon, the cyanide content is substantially lower and usually is about 10% and barium chloride in a quantity of about 50 to 55% is the main constituent of the salt bath. The customary working temperature of such accelerated baths is 930° C. and it is impossible in general to employ them at higher temperatures to accelerate the carburization and the depth thereof, as cyanide losses which are not feasible occur at higher temperatures.

The cyanide losses occur by burning off and, more important, by decomposition of the cyanide with the formation of alkaline compounds, especially sodium carbonate and sodium oxide. These decomposition products evidently deter the decomposition of the cyanide which is required for the cementing action and can upon accumulation in the bath hinder a satisfactory course of the cementation even though the baths contain sufficient cyanide.

Many attempts have been made to overcome this difficulty by adding accelerators of the most varied types to the baths, for example, compounds of metals, such as their halides, which form cyanides which decompose more readily than alkali metal cyanides. All of these attempts, however, have not led to carburization processes which can be carried out at temperatures above 930° C., even though the carburization velocity and depth was not always satisfactory. The high cyanide losses, as well as the accumulation of carburization deterring decomposition products which cannot be completely compensated for by continued replenishment of the baths with salts, have prevented technicians from attempting to carburize with fused cyanide containing salt baths at temperatures in excess of 930° C. worth mentioning.

According to the invention, it was unexpectedly found

2

that carburization could be carried out with fused salt baths primarily composed of alkaline earth metal halides and cyanides at temperatures considerably higher than previously customarily used with increased velocity and intensity of the carburization if care is taken that the alkaline earth metal halide content in such baths is constantly maintained above 75% and preferably at about 85%. The cyanide content of such baths can be about the same as in the normal accelerated baths, that is, around 10%. It was unexpectedly found that with the baths according to the invention, even when temperatures of above 950° C., for example 1000 to 1100° C., are employed for the carburization, the deleterious decomposition of the cyanide is no greater than with the normal baths containing 50 to 55% of barium chloride operated at temperatures up to 930° C. The small losses of cyanide occurring during use of the baths according to the invention can be compensated for by replenishing the baths with a salt mixture of corresponding composition.

15 The advantages of the baths according to the invention become especially apparent when carburization temperatures between about 1000 and 1100° C. are employed. Expediently, salt mixtures consisting of 75 to 95% of alkaline earth metal halide, especially barium chloride, and 25 to 5% of sodium cyanide are employed to prepare the baths for carrying out the carburization process according to the invention. For example, when a salt mixture composed of 90% barium chloride and 10% of sodium cyanide was fused and used for carburization of iron or steel, it assumed the following composition after continued use with replenishment with a mixture of 4 parts of barium chloride and 1 part of sodium cyanide:

20

|                                 | Percent |
|---------------------------------|---------|
| 35 BaCl <sub>2</sub>            | 87      |
| NaCN                            | 6       |
| Na <sub>2</sub> O               | 4       |
| Na <sub>2</sub> CO <sub>3</sub> | 1.8     |
| NaCl                            | 1.3     |

25 In contrast, a known bath for carburization at 930° C., hereinafter termed C-5 bath, had the following complicated composition right from the start:

|                      | Percent |
|----------------------|---------|
| 45 BaCl <sub>2</sub> | 54      |
| SrCl <sub>2</sub>    | 3.5     |
| NaCN                 | 9.4     |
| BaCO <sub>3</sub>    | 1.4     |
| NaCl                 | 11.8    |
| KCl                  | 20      |
| C                    | 0.1     |

30 In continued use of such a bath, it must be replenished with an admixture of 2 parts of a mixture of the same composition as the original bath and 1 part of sodium cyanide. Consequently, considerably more sodium cyanide is required for replenishing this known bath than for the bath according to the invention where, for example, as described above, a mixture of 4 parts of barium chloride and 1 part of sodium cyanide can be employed.

35 After continued operation with the C-5 bath at 930° C., considerable quantities of deleterious sodium carbonate can accumulate and can amount to 24.2% with a barium chloride content of 50% and a sodium cyanide content of 10%.

40 Aside from the advantages of simpler composition of the baths according to the invention and more economical NaCN replenishing requirements, it was found that the baths according to the invention could be operated at temperatures over 950° C., for example, between 1000 and 1100° C., without undue cyanide losses and effect an unexpected increase in carburization velocity and case

45

50

55

60

65

70

depth, especially at the higher range of temperatures mentioned.

The accompanying drawings serve to illustrate the beneficial effects attainable with the carburizing baths according to the invention.

Fig. 1 of the drawings shows a graph giving the relationship between the carburization depth and the carburization time when operating with a bath according to the invention and with the C-5 bath.

Fig. 2 of the drawings shows a graph giving the carbon content at various depths of the case obtained with a bath according to the invention and with the C-5 bath.

Referring to Fig. 1, curves A, B and C represent the carburization depth corresponding to a 0.3% carbon content obtained with test rods of 0.5% C-steel. Curve A represents the results obtained with the C-5 bath operated at 930° C., whereas curves B and C represent the results with a bath according to the invention of 90% BaCl<sub>2</sub> and 10% NaCN, hereinafter termed bath C-8, operating respectively at 1050° C. and 1100° C. As can be seen from curve A, a carburization depth greater than 2.5 mm. can hardly be expected using the C-5 bath even with an infinite carburization time and, with carburization times of 6 to 10 hours, which are commercially feasible, a carburization depth of 2 mm. is not even achieved. On the other hand, it can be seen from curves B and C, with the bath according to the invention a carburization depth of 1.9 mm. is attained after only 4 hours' carburization at 1050° C. and a carburization depth of 2.5 mm. is attained after only 4 hours' carburization at 1100° C.

For further comparison, the following table gives the carburization depths in mm. taken from the curves in Fig. 1:

| Bath | Temp.,<br>° C. | Carburization time in hours |      |      |      |
|------|----------------|-----------------------------|------|------|------|
|      |                | 2                           | 4    | 10   | 16   |
| C-5  | 930            | 1.8                         | 1.25 |      |      |
| C-8  | 1,050          | 1.30                        | 1.9  | 3.05 | 3.90 |
| C-8  | 1,100          | 1.65                        | 2.5  | 4.4  | 5.70 |

As shown in such table, the process according to the invention renders it possible to obtain carburization depths which were not considered possible with the previously employed processes with the customary baths.

The relationship of the carbon content with increase in carburization depth also indicates the superiority of the process and salt baths according to the invention.

In Fig. 2, curves D, E and F represent the carbon content at various depths in the case obtained after 4 hours' carburization of test rods of C-15 steel. The carbon contents at such various depths were ascertained by machining off successive layers of the case and subjecting the resulting turnings to chemical analysis. Curve D represents the results obtained with the C-5 bath operated at 930° C. Curves E and F represent the results obtained with bath C-8, respectively operated at 1050° C. and 1100° C.

The following table gives the carbon content at depths of 1 mm. and 2 mm. taken from the curves of Fig. 2:

| Bath | Temp.,<br>° C. | Carburization depth |                 |
|------|----------------|---------------------|-----------------|
|      |                | 1 mm.               | 2 mm.           |
| C-5  | 930            | Percent<br>0.41     | Percent<br>0.16 |
| C-8  | 1,050          | 0.68                | 0.25            |
| C-8  | 1,100          | 0.78                | 0.43            |

These values clearly indicate the unexpectedly high carburization action which is obtained with the barium chloride rich baths according to the invention. For example, in the relatively short carburization of 4 hours' duration, the same carbon content as is achieved with the known C-5 bath at 1 mm. depth is achieved at twice the depth with bath C-8.

The process according to the invention, especially when employing higher carburization temperatures, has been found particularly suited for the carburization of ferrous metal articles subject to wear wherein a great depth of hardness is desired, for example, for mining chains, caterpillar tractor and excavator parts, and also parts of large engines, such as locomotives and marine diesels.

It is, of course, to be understood that the salt mixtures employed as carburizing baths according to the invention can contain other usual additions, such as accelerators or carburization regulators, in addition to the barium chloride and sodium cyanide. However, accelerators are usually not required in view of the higher carburization temperatures which can be employed.

The process according to the invention is advantageously carried out in furnaces provided with ceramic lined containers for the fused salt baths. It has furthermore been found advantageous to provide arched pressure resistant surfaces on the sheet metal cladding for the ceramic lining, especially on the covering plate for the ceramic lining, in order to prevent the ceramic bricks from being lifted up by the salt melt penetrating the joints between the bricks, especially during the heating up or cooling off of the salt baths.

I claim:

1. A method of carburizing ferrous metals which comprises introducing such ferrous metals into a fused salt bath essentially consisting of a fusion of a mixture of 75 to 95% of barium chloride and 25 to 5% of an alkali metal cyanide maintained at a temperature of at least 1000° C.

2. A method of carburizing ferrous metals which comprises introducing such ferrous metals into a fused salt bath essentially consisting of a fusion of a mixture of 75 to 95% of barium chloride and 25 to 5% of a sodium cyanide maintained at a temperature between 1000° C. and 1100° C.

3. The process of claim 2 in which said fused salt bath contains at least 85% of barium chloride.

#### References Cited in the file of this patent

#### UNITED STATES PATENTS

|              |                 |               |
|--------------|-----------------|---------------|
| 1,980,152    | Beck et al      | Nov. 6, 1934  |
| 2,007,136    | Albrecht et al. | July 2, 1935  |
| 2,049,806    | Holt            | Aug. 4, 1936  |
| 2,339,223    | Holt            | Jan. 11, 1944 |
| 55 2,342,104 | Holt            | Feb. 22, 1944 |

#### FOREIGN PATENTS

|         |               |              |
|---------|---------------|--------------|
| 204,759 | Great Britain | Oct. 1, 1923 |
|---------|---------------|--------------|

#### OTHER REFERENCES

60 "Molten Salt Baths for Heat Treatment and Case Hardening of Steel," published by E. I. du Pont de Nemours & Co. (Inc.), June 7, 1946, pp. 33, 34.